

1

2,825,644

PROCESS OF REMOVING LEAD FROM COPPER  
BASE ALLOYS

Paul Kemp, Bois Colombes, France

No Drawing. Application January 28, 1954  
Serial No. 406,886

5 Claims. (Cl. 75—128)

The present invention relates to the process of removing lead from finely divided copper base alloys such as turnings and grindings.

A purpose of the invention is to remove lead from finely divided scrap of copper base alloys so as to permit the scrap to be remelted in order to produce ingots which are relatively low in lead.

A further purpose is to eliminate lead from particles of copper base alloy by treatment with nitric acid as substantially the only reagent, thus minimizing the solution of copper and other ingredients, operating preferably at room temperature and in a concentration range of 2 to 13 percent of concentrated nitric acid in water by volume.

A further purpose is to employ a counter current treatment of the particles of copper base alloy, first with weak nitric acid and then with stronger nitric acid.

A further purpose is to degrease the particles of copper base alloy, prior to treatment with the nitric acid.

A further purpose is to agitate the nitric acid and the copper base alloy particles during the treatment.

A further purpose is to recover the lead from the solution by precipitation.

Further purposes appear in the specification and in the claims.

The removal of undesirable elements from alloys is usually accomplished by fusion of the alloy, followed in some cases by oxidation or volatilization of elements to be eliminated. In other cases, fractional solidification is employed to eliminate undesired elements, which are concentrated in one of the fractions obtained. In still other instances, substances are added with which the base alloying material forms insoluble compounds.

It is not always possible however to employ thermal processes. Aluminum, zinc or iron can be removed from copper base alloys by one of these methods, but it is not possible at the present time to decrease the lead content even to a slight extent without at the same time losing a large part of the tin.

The elimination of lead from such alloys is, however, an important problem when it is considered that many specifications for bronzes of high quality permit very small lead contents. It has, therefore, in many cases been necessary to make such high quality bronzes from virgin copper and tin. The use of secondary bronze from scrap has not been permitted because such material has too high a content of lead. It is therefore necessary to find some other process to solve this problem.

Metallic alloys are essentially composed of metallic crystals, solid solutions and intermetallic compounds. The differences between these various constituents are readily recognizable under the microscope. It is thus theoretically possible to eliminate a certain constituent by a wet process, treating the alloy with a reagent which is capable of dissolving the desired constituent without attacking the rest of the alloy.

Lead is of course practically insoluble in copper alloy in the solid state, and it appears as a distinct phase in

2

the micro-structure of bronze and brass. The elimination of lead by a wet process is then possible in alloys which are sufficiently finely divided to be attacked in depth.

It has already been proposed to employ certain organic compounds such as tartarates or citric acid in combination with nitric acid to remove lead from grindings or turnings of bronze. This process has not been satisfactory, and in any case it is necessary to have an apparatus having a lining of special material and to operate at a temperature of about 100 C.

Lead has also been eliminated by double decomposition with salts of copper in acid solution. Such copper salts are relatively expensive. Copper deposits on the material under treatment in the course of the reaction and to a certain extent retards the penetration of the reacting materials into the interior.

In accordance with the present invention, lead is removed from copper alloys and particularly finely divided copper base alloys such as turnings and grindings of brass and bronze, by a reaction with nitric acid alone.

Nitric acid is in the present process the only reactant. When one realizes that nitric acid not only attacks lead but also attacks copper and zinc, and is used in analytical laboratories to dissolve bronze and brass, it will be appreciated that the use of nitric acid alone to dissolve lead from a copper base alloy is very remarkable. The present inventor has discovered that by observing certain precautions as indicated herein, it is possible to eliminate the lead without dissolving the slightest trace of copper.

20 The process of the present invention has the advantage that the price is low. Another great advantage of the present process is that operation is possible at ambient temperature and in fact is preferably carried on at such temperatures. Thus, a better result is obtained than by previous processes, using a very simple installation and at low cost.

25 The concentration of the acid to be employed depends in part upon the material to be treated. Generally speaking, good results have been obtained, using concentrations of from 2 to 13 percent of nitric acid in water by volume. Higher concentrations are preferably used at lower temperatures (below 20° C.) and lower concentrations are preferably used at higher temperatures such as are encountered in summer.

30 It is preferable to start out a deleading operation using an acid which has previously been used in deleading an earlier charge. The last residual content of lead is preferably eliminated by fresh and more concentrated nitric acid.

35 Bronze turnings in practice almost always are coated with oil or grease. It has been found that the elimination of lead can be accomplished most effectively if the turnings have previously been subjected to a treatment which removes this grease coating suitably by heating above the point of decomposition of the grease, or by degreasing the turnings with a solvent.

40 In order to secure a rapid and complete reaction, it is desirable to mix the turnings intimately with the acid. A simple means of mixing is to carry out the process in a rotating drum containing the finely divided copper base alloy. The drum can be constructed of wood which is quite resistant to the treatment.

45 Depending upon the nature of the copper base alloy particles, the lead will be more or less completely removed. On the average 70 to 80 percent by weight of the lead content is eliminated when ordinary turnings of brass or bronze are used, and 95 percent by weight is eliminated from grindings or very fine turnings.

50 To recover the lead, the solution containing the lead can be neutralized, for example by lime or by a carbonate, and the total quantity of lead is then recovered as a hydroxide or carbonate substantially free from other

metals. The appropriate lead compound is easily reduced to metallic lead.

*Example I*

1000 kilograms of bronze turnings of the following composition by weight:

|        | Percent |
|--------|---------|
| Tin    | 6.7     |
| Copper | 84.3    |
| Lead   | 4.6     |
| Zinc   | 4.3     |

are charged into a rotating drum which is filled with a mixture of 640 liters of water and 60 liters of concentrated nitric acid. The drum is turned for 90 minutes at a temperature of 18° C., and the solution is then emptied. The solution when emptied contains 50 grams of lead per liter. The turnings after the treatment have the following analysis by weight:

|        | Percent |
|--------|---------|
| Tin    | 6.9     |
| Copper | 87.7    |
| Lead   | 1.0     |
| Zinc   | 4.2     |

The recovery from the treatment amounts to 964 kilograms of alloy.

*Example II*

1000 kilograms of leaded bronze turnings of the following analysis by weight:

|        | Percent |
|--------|---------|
| Tin    | 7.5     |
| Copper | 75.8    |
| Lead   | 14.7    |
| Zinc   | 1.8     |

are treated with the leaded solution remaining from the treatment of Example I. The treatment with this solution is continued for 30 minutes, and then the solution is emptied, at which time it contains 85 grams of lead per liter. The drum is then charged with a new solution of 640 liters of water and 60 liters of nitric acid. This new solution is used to treat the turnings with agitation in the drum for one hour, after which the new solution is removed and the turnings are dried. The recovery of turnings is 870 kilograms having the following composition by weight:

|        | Percent |
|--------|---------|
| Tin    | 8.6     |
| Copper | 87.0    |
| Lead   | 2.3     |
| Zinc   | 2.1     |

From the two solutions obtained from this example,

160 kilograms of lead were recovered by precipitation in the form of hydroxide.

It will be evident that the process of the invention has wide application particularly in secondary copper refining especially to produce secondary ingots of precise analysis.

In view of my invention and disclosure variations and modifications to meet individual whim or particular need will doubtless become evident to others skilled in the art, to obtain all or part of the benefits of my invention without copying the process shown, and I, therefore, claim all such insofar as they fall within the reasonable spirit and scope of my claims.

Having thus described my invention what I claim as new and desire to secure by Letters Patent is:

1. The process of removing lead from finely divided copper base alloys, which comprises treating the particles of copper base alloy with a water solution of 2 to 13% of nitric acid by volume in which nitric acid is the only reagent present.

2. The process of claim 1, in which the treatment is at ambient temperature.

3. The process of claim 1, in which the treatment is carried on first with partially spent nitric acid solution and then with a stronger concentration of nitric acid solution.

4. The process of claim 1, in which the particles of copper base alloy and the nitric acid solution are agitated during treatment.

5. The process of claim 1, in which the lead is subsequently recovered from the solution by precipitating as a salt of the class consisting of a hydroxide and a carbonate.

**References Cited in the file of this patent**

**UNITED STATES PATENTS**

|           |             |                |
|-----------|-------------|----------------|
| 1,192,945 | Sherwood    | Aug. 1, 1916   |
| 1,375,930 | Ralston     | Apr. 26, 1921  |
| 1,643,922 | Christensen | Sept. 27, 1927 |
| 1,918,817 | Mantell     | July 18, 1933  |
| 2,342,733 | Guyard      | Feb. 29, 1944  |

**FOREIGN PATENTS**

|           |        |                |
|-----------|--------|----------------|
| 1,051,683 | France | Sept. 16, 1953 |
|-----------|--------|----------------|

**OTHER REFERENCES**

Serial No. 409,751, Guyard (A. P. C.), published May 4, 1943.

Engineering Metals and Their Alloys, by Samans. Published in 1952 by The Macmillan Co., N. Y., pages 12, 15 and 16.

Corrosion Handbook, by Uhlig. Published in 1948 by John Wiley and Sons Inc., N. Y. Pages 66, 67, 77, 100, 101 and 213.

Metals Handbook, 1948 edition. Published by The American Society for Metals, Cleveland, Ohio. Page 1200.